

## UNITED STATES PATENT OFFICE

2,360,784

## METALLIC COATING ALLOY

Arthur J. Mauger, Gary, Ind., and Alfred H. Ward, Brentwood, Pa., assignors to Carnegie-Illinois Steel Corporation, a corporation of New Jersey

No Drawing. Application May 1, 1942,  
Serial No. 441,358

## 5 Claims. (Cl. 75—178)

In accordance with the present invention, there are provided certain improvements in metal coating compositions of the kind that are employed for producing the so-called "galvanized" coatings on a ferrous metal base.

It is highly desirable in galvanizing operations to produce a coating which is characterized by the appearance of spangles. Also, it is desirable to employ in the coating compositions elements which increase the fluidity of the galvanizing bath.

Heretofore it has been the general practice in hot dip zinc coating processes, such as those commonly referred to as "galvanizing," to use additions of metallic tin to the molten coating bath to improve the fluidity, and to provide a suitable set of conditions for producing a distinctive spangled finish. The benefits derived from such additions of tin to the coating baths have been described as being due to a beneficial influence of the tin on the surface tension properties during solidification of the coating, or to a prolongation of the freezing period caused by the presence of a tin-zinc eutectic. The characteristic finish resulting from the practice embodies a relatively smooth finish with an even distribution of the coating on the surfaces of the coated article. Without the addition of tin, the zinc coating tends to form unevenly from place to place on the object and individual units of crystallization in the solidified coating are separated by a network of depressed boundary lines where the coating is relatively thin. In these thin areas, the protection afforded by the coating is less than that in the major portion of the surface where the coating is heavier. The addition of tin, in amounts of from substantially 0.25% to 1.00% or even in larger quantities, causes the elimination of these depressed boundaries.

The multitudinous applications of galvanized products are too well-known to require comment; and it is obvious immediately that the desirability of obtaining a satisfactory protective coating is of high importance. However, because of the immediate scarcity of tin, and its high strategic value, the use of tin in galvanizing baths has become prohibitive.

Consequently, it is of high importance to find substitutes for tin in this particular application, which substitutes will not be prohibitive either from the standpoint of economics or from the standpoint of strategic availability.

Consequently, the present invention is predicated upon investigations leading to the finding

of suitable additional agents to galvanizing baths which will perform the functions of tin at least as satisfactorily as does tin itself.

In the investigations leading up to the present invention, it has been determined that metallic lead, which is present as a constituent impurity in the grade of zinc (known in the trade as "Prime Western Spelter") used in galvanizing operations, is responsible for the depressed boundaries described above herein. Also, the investigations leading to the present invention have established that the depth of these depressions is roughly proportional to the lead content of the coating. But, since lead imparts a certain degree of fluidity to the bath and also promotes the formation of spangles in the coating, the presence of lead in the bath, instead of being regarded as detrimental in view of the foregoing, is in fact highly desirable. The investigations leading to the present invention show further that the minimum amount of lead above which attractive spangles can be produced is about 0.20%. Spangles increase in size roughly proportional to the lead content until the amount of lead reaches about 1.00%. At this percentage the depressions around the spangles are pronounced.

Additionally, the investigations leading to the present invention establish that metallic cadmium when present in the spelter bath in amounts greater than 0.05% tends to promote the formation of "frosty" spangles and to minimize objectionable depressions at the spangle boundaries. This tendency is found to increase with the cadmium content of the bath up to about 1.00%. The finish produced with cadmium alone, however, is not as attractive or uniform as that of tin-bearing baths.

The investigations leading to the present invention further establish that antimony in amounts greater than 0.05% promotes the formation of the decorative spangles even in the absence of other alloying constituents. However, unless other additions are present, the crystalline growth during solidification is such as to result in extremely rough surfaces with portions of the spangles drawn up above other portions.

In accordance with the present invention, therefore, it is found that with additions of the alloying metals, lead, cadmium and antimony, to the galvanizing bath, there may be utilized all the desirable functions of each metal, and there is obtained a galvanizing bath with a fluidity equal to or better than that produced by the addition of tin. Furthermore, in accordance with the

present invention, it has been found that the disadvantageous effects of the individual metals are materially modified satisfactorily so that there are produced from the improved bath, coatings which are of equal uniformity and appearance produced by the addition of tin, and the coating composition is usable in any standard coating equipment without changing any of the established practices of cleaning, pickling, or fluxing in any way. The desirable results of the present invention are obtained without the use of tin, and the composition of the bath is such that strategic scarcity of metals employed is obviated.

In practicing the present invention, to commercial "Prime Western" zinc containing substantially 0.70% of lead and up to 0.20% cadmium, there is added sufficient high purity zinc of electrolytic or equivalent grade to reduce the lead content of the bath to the desired range of 0.25% to 1.00%. To this bath then is added sufficient cadmium metal to obtain a cadmium content of from 0.2% to 1.00%. As an alternative to such procedure there may be utilized the first drawn condensate from zinc retorts which may contain a low lead content of about 0.30% to 0.50%, and a high cadmium content of about 0.25% to 0.35%. This grade of material may or may not contain traces of residual tin up to 0.01%.

To either material there is added sufficient antimony in the form of a zinc-antimony or lead-antimony alloy to build up an antimony content of from 0.05% to 0.30%, the preferred range of composition being lead, 0.50% to 1.00%; cadmium, 0.30% to 0.50%; and antimony 0.05% to 0.20%.

We claim:

1. A bath for hot dip galvanizing, which consists of zinc containing from approximately 0.5% to approximately 1% lead, from approximately .20% to approximately .50% cadmium, 40 and from approximately 0.05% to approximately 0.2% of antimony.

5. A tin-free bath for hot dip galvanizing, having properties of fluidity when molten and also having coating properties at least comparable to corresponding properties of a zinc-tin galvanizing bath containing at least 0.25% tin, the said tin-free bath being consisting of principally zinc together with small but effective amounts of lead, cadmium and antimony.

3. A tin-free bath for hot dip galvanizing, having properties of fluidity when molten and also having coating properties at least comparable to corresponding properties of a zinc-tin galvanizing bath containing at least 0.25% tin, the tin-free bath being consisting of zinc, together with 10 small but effective amounts of lead, cadmium, and antimony, wherein the lead predominates over the cadmium and antimony.

4. A tin-free bath for hot dip galvanizing, having properties of fluidity when molten and also 20 having coating properties at least comparable to corresponding properties of a zinc-tin galvanizing bath containing at least 0.25% tin, the tin-free bath being consisting of zinc together with small but effective amounts of lead, cadmium and antimony, and wherein the lead is present in 25 from approximately 0.5% to approximately 1% lead, the lead predominating over the cadmium and antimony.

5. A tin-free bath for hot dip galvanizing, having properties of fluidity when molten and also 30 having coating properties at least comparable to corresponding properties of a zinc-tin galvanizing bath containing at least 0.25% tin, the tin-free bath being consisting of zinc together with small but effective amounts of lead, cadmium, and antimony, wherein the lead does not exceed 35 approximately 1% and predominates over the cadmium and antimony, there being less antimony than cadmium.

ARTHUR J. MAUGER.  
ALFRED H. WARD.